

# UNITED STATES PATENT OFFICE.

JULIUS RÜTTERS, OF BERLIN, GERMANY; ANDREAS COLLSTROP, OF COPENHAGEN, DENMARK, AND FRITZ NOEBE AND GUSTAV KRAEMER, OF BERLIN, GERMANY, EXECUTORS OF SAID RÜTTERS, DECEASED.

## PROCESS OF IMPREGNATING WOOD.

No. 894,061.

Specification of Letters Patent.

Patented July 21, 1908.

Application filed May 20, 1903. Serial No. 157,934.

*To all whom it may concern:*

Be it known that I, JULIUS RÜTTERS, manufacturer, a subject of the Emperor of Germany, and resident of Berlin W., Prussia, 5 German Empire, have invented an Improved Process for the Impregnation of Wood, of which the following is a specification.

In the ordinary process of impregnating wood, the wood after the air has been extracted from it more or less completely by means of a vacuum, is treated with the impregnating liquid or liquids by means of hydraulic pressure until the pores of the wood have been filled or nearly filled, the object 15 being to introduce into the wood as much impregnating liquid as possible, after which the wood was considered ready for use. This method has the defect, that the large quantity of impregnating liquid absorbed by 20 the wood renders it unnecessarily heavy and increases the expense of the treatment.

The present invention has for its object, to effect the complete impregnation of the wood by means of a comparatively small quantity 25 of impregnating liquid distributed in all cellulas throughout the wood up to the core. For this purpose the wood to be treated is placed in the impregnating cylinder or other closed receptacle, after which the impregnating liquid, such as tar oil or the like, which 30 may be cold or warm, is caused to enter the cylinder until the cylinder is quite full. Subsequently pressure is applied until the desired quantity of the impregnating liquid 35 has entered the wood, after which the pressure is taken off and the excess of impregnating liquid drawn off or discharged from the cylinder. Thereupon the wood lying in the cylinder is subjected to the action of saturated or superheated steam (up to 4 atmospheres) or of hot gases under pressure or

of a mixture of steam and hot gases under pressure, for a period depending on the nature and thickness of the wood (usually from 1 to 3 hours). Under the influence of heat 45 and pressure the impregnating liquid which has been forced into the wood, is caused to penetrate it up to the core.

As mentioned above, the improved process requires much less impregnating liquid than 50 the process generally employed, moreover it may be carried out without any alteration of the plant hitherto employed. After the impregnation has been completed, the surface of the wood is clean and the impregnating 55 liquid is not liable to sweat out.

Having now described my invention, I claim:

1. The herein described process of preserving wood, which consists in immersing 60 the wood in tar-oil, subjecting the tar oil with the wood to pressure, introducing an amount of tar-oil into the wood insufficient for filling all pores of the wood, drawing off the tar-oil surrounding the wood and introducing a hot 65 gaseous fluid under pressure into the wood.

2. The herein described process of preserving wood, which consists in immersing the wood in tar-oil, subjecting the tar-oil with the wood to pressure, introducing an amount 70 of tar-oil into the wood insufficient for filling all pores of the wood, drawing off the tar oil surrounding the wood and introducing steam under pressure into the wood.

In testimony, that I claim the foregoing as 75 my invention, I have signed my name in presence of two subscribing witnesses.

JULIUS RÜTTERS.

Witnesses:

FRITZ NOEBE,  
EMIL FLOER.